# EUROPEAN PATENT SPECIFICATION

(11) **EP 0 597 179 B1**
(45) Date of publication and mention of the grant of the patent: **09.04.1997**
(21) Application number: 93109326.4
(22) Date of filing: 10.06.1993
(51) Int. Cl.: G03C 7/407, G03C 7/413, G03C 7/42

(54) **Method for processing a silver halide color photographic light-sensitive material**
Verfahren zur Behandlung eines farbphotographischen lichtempfindlichen Silberhalogenidmaterials
Procédé de traitement d'un matériau photographique couleur à l'halogénure d'argent sensible à la lumière

(30) Priority: 19.06.1992 JP 161336/92
(43) Date of publication of application: 18.05.1994
(73) Proprietor: KONICA CORPORATION, Tokyo 163 (JP)
(72) Inventor: Satake, Wataru, c/o Konica Corporation, Hino-shi, Tokyo (JP)
(74) Representative: Türk, Gille, Hrabal, Leifert

(56) References cited:
- EP-A- 0 361 407
- EP-A- 0 411 502
- EP-A- 0 439 142
- EP-A- 0 475 768

## Description

### FIELD OF THE INVENTION

The present invention relates to a method for processing a silver halide color photographic light-sensitive material, particularly to a method for processing a silver halide color photographic light-sensitive material which exhibits an excellent processing stability even in low-replenishment processing or rapid processing.

### BACKGROUND OF THE INVENTION

Basically, the processing of a light-sensitive material comprises the two processes of color development and desilverization, and the desilverization comprises a bleaching process and a fixing process, or a bleach-fixing process. A rinsing process and a stabilizing process are added thereto as additional processes.

In the color developing process, an exposed silver halide is reduced to silver and, at the same time, an oxidized aromatic primary amine developing agent reacts with a coupler to form a dye. During this process, halogen ions formed by the reduction of a silver halide are dissolved and accumulated in the color developer. In addition, components contained in a silver halide photographic light-sensitive material, such as inhibitors, are also dissolved and accumulated in the developer. In the desilverizing process, the silver formed in the developing process is bleached by an oxidizing agent and, then, all the silver salts are removed in the form of soluble salts from the photographic light-sensitive material with the aid of a fixing agent. These bleaching process and fixing process can also be carried out simultaneously by use of the monobath bleach-fixing process.

As described above, development-inhibiting materials are accumulated in the color developer during the development of a photographic light-sensitive material; on the other hand, the color developing agent is consumed or taken out of the color developer by accumulating in the photographic light-sensitive material and, as a result, its component concentration continues to decrease.

In the bleach-fixer, silver salts and halogen ions dissolved out of a light-sensitive material accumulate, and the bleach-fixer itself is diluted to a lower component concentration by a solution brought in from the preceding bath.

Accordingly, in order to avoid fluctuations in development results due to fluctuations in concentrations of developer components, any developing method which processes a large amount of silver halide photographic light-sensitive materials by use of an automatic processor cannot dispense with a means to keep the concentration of each color developer component within a prescribed range.

As a usual manner to carry out such a means, a developer is replenished to make up for deficient components and dilute the increment of unnecessary components. This replenishment of a developer inevitably yields a large amount of waste overflow and, thereby, causes serious problems in processing cost and environmental protection. Therefore, there have been proposed and put to practical use, in recent years, a method of regenerating a developer by use of ion exchange resins or electrodialysis, a method of replenishing a concentrated solution, and a method of reusing an overflow as a replenisher by adding a regenerant thereto.

The regeneration of a developer can be carried out by removing bromides, unnecessary accumulated components, and replenishing lacking components. But this method (comprising ion exchange or electrodialysis) has a disadvantage that the characteristics of a developed light-sensitive material is degradated unless the concentrations of developer components are kept constant by means of chemical analyses which need complicated procedures; therefore, it can hardly be carried out in small processing laboratories including the so-called mini-laboratories which have no special skill. In addition, it has another disadvantage of high initial cost.

Though not much skill is needed in the method of reusing an overflow as a replenisher by adding a regenerant, it requires a site for installing a stock tank, etc. and is troublesome to carry out in many processing laboratories. Accordingly, this method is also difficult to introduce into small laboratories.

In contrast with these methods, the method of replenishing with a small amount of concentrated solution is suitable for small laboratories, because it needs no new installations and is easy to carry out. However, this method has some problems, too. For example, in such a small volume replenishment of a color developer, matters dissolved out of light-sensitive materials are accumulated in large amounts and, in addition, decomposition products produced by air oxidation of developer components are also accumulated in large amounts. For a bleach-fixer, the concentration of contaminants increases in a front tank and, as a result, decomposition and accumulation of the contaminants amount to an undesirable level. Primary undesirable effects caused by such phenomena are fluctuations in pH during processing, which deteriorate the processing results, and undesirable influences of the decomposed products on light-sensitive materials.

There are spreading processing laboratories called 1-hour photos, which do business with the catch phrase of 1-hour finish and further 30-minute finish. This tendency is becoming stronger in recent years, and delivery in a much shorter time is desired. Such a fast delivery inevitably promotes on-the-spot processing as well as downsizing and improving efficiency of automatic processors and, thereby, facilitates the start of photographic processing business at tourist spots, camera shops, drugstores and convenience stores in addition to existing mini-laboratories; this needs a further shortening of the processing time.

Such ultrarapid processing requires that bleach-fixing be completed in a short time by rapidly exchanging components brought from the preceding bath for bleach-fixing components in component layers of light-sensitive material. Further, in the bleach-fixing process, prevention of stains and improvement in recoloring property of color image have, in particular, been desired for the achievement of such small volume replenishing and ultrarapid processing. In the specification, "recoloring property" means an ability of recoloring of dye image in a bleaching solution by converting leuco-dye contained in a developed dye image to colored dye by oxidation.

Addition of a large amount of bromide ions has so far been a usual preventive measure against stains, but it is not so effective and has a problem of rusting processing tanks. Further, use of high concentration bleach components, a usual means to improve the recoloring property, is not desirable in respect of environmental pollution and deposition of solid matters at low temperatures.

EP-A-0 411 502 describes a method for processing a silver halide color photographic material with a color developer containing a hydroxylamine compound by using an automatic processor. The hydroxylamine compound comprises as a functional group a carboxyl group, a sulfo group, a phosphono group, phosphinic acid residue, a hydroxyl group, an amino group, an ammonio group, a carbamoyl group, a sulfamoyl group or an alkyl sulfonyl group. The use of monosaccharides for the color developer is not described. The content of silver chloride in at least one emulsion is preferably 90 mole % or more. In the examples the composition of the bleach-fixing solution comprises iron(III)ammonium ethylenediaminetetraacetate. According to this document the opened surface ratio of the color developer in the tank of the automatic processor is decisive for obtaining a stable photographic performance wherein the fluctuation and gradation due to continuous processing is suppressed. The use of selected aliphatic dibasic acids in the bleach-fixing solution is not disclosed.

EP-A-0 361 407 discloses a method for processing silver halide color photographic materials. The color developing solution can contain monosaccharides. A layer having a silver chloride content of 97 mole % is described. Organic Fe(III) complex salts such as salts of ethylenediaminetetraacetic acids, diethylenetriaminepentaacetic acids or organic acids such as tartaric acid or malic acid are used in the bleach-fixing solution. The combined use of Fe(III) salts and organic acids in the bleach-fixing solution is not disclosed.

EP-A-0 475 768 describes a method for processing a silver halide color photographic material. Therein, the hydroxylamine compounds containing hydroxyl, sulfo acid and carboxyl groups, respectively are disclosed as ingredients for the color developer. The content of silver chloride in the emulsion layers is described to be preferably not less than 80 mole %. The bleaching solution contains ferric complex salts such as ferric ethylenediaminetetraacetate, ferric dieethylenetriaminepentaacetate, ferric 1,2-cyclohexanediamine-tetracetate or ferric glycoletherdiaminetetraacetate. Furthermore, the bleacher can contain aliphatic dibasic acids. However, according to this document bleaching and fixing are carried out in separate steps.

EP-A-0 439 142 describes a composition for color development in a method for processing a silver halide color photographic material. The developer can contain hydroxylamine compounds. The photographic material contains 80 mole % or more of silver chloride. The bleach-fixing solution comprises Fe- complex salts of e.g. ethylenediaminetetraacetic acids,
glycoletherdiaminetetraacetic acids or cyclohexanediaminetetraacetic acids. Iron(II) complexes are preferred. Tartaric acid may be contained as a buffering agent in the bleach-fixing solution. However, use of further aliphatic dibasic acids and the specific effects thereof are not described in this document.

### SUMMARY OF THE INVENTION

Accordingly, the object of the present invention is to provide a method for processing silver halide color photographic light-sensitive materials which causes neither stains nor recoloring failure in the photographic material even when applied to rapid processing or small volume replenishing.

The object of the invention is achieved by a method for processing a silver halide color photographic light-sensitive material. The method comprises the steps of
developing a silver halide color photographic light-sensitive with a color developer, and
bleach-fixing the light-sensitive material with a bleach-fixer. In the above, a silver halide emulsion layer of the light-sensitive material comprises silver halide grains having a silver chloride content of not less than 80 mol %; the color developer contains a compound represented by the following Formula I or a monosaccharide; and the bleach-fixer contains a ferric complex salt of aminopolycarboxylic acid selected from the following Group 1 and a aliphatic dibasic acid selected from the following Group 2;
wherein L is a substituted or unsubstituted alkylene group; A is a carboxyl group, a sulfo group, a phosphono group, a phosphinic acid group, hydroxyl group, an amino group, an ammonio group, a carbamoyl group or a sulfamoyl group, in which the amino group, ammonio group, carbamoyl group and sulfamoyl group each may have an alkyl group as a substituent; R is a hydrogen atom or a substituted or unsubstituted alkyl group;
Group 1
   Ferric ethylenediaminetetraacetate,
   Ferric ethylenetriaminepentaacetate,
   Ferric trans-1,2-cyclohexanediaminetetraacetate,
   Ferric β-alaninediacetate,
   Ferric ethylenediaminedisuccinate,
   Ferric nitrylotriacetate,
   Ferric N-hydroxyethylethylenediaminetriacetate and
   Ferric glycoletherdiaminetetraacetate;
Group 2
   Oxalic acid,
   Succinic acid,
   Maleic acid,
   Fumaric acid, and
   Adipic acid.
Using the compound represented by formula I in a color developer and using an aliphatic dibasic acid in a bleach-fixer are known to those skilled in the art. It was further known to use iron complexes with an aminopolycarboxylic acid in a bleaching or bleach-fixing solution together with tartaric acid as a buffering agent. However, it was an unexpected finding that a stable, stain-free and high-recoloring processing method could be achieved for the first time by combining the above compounds and by utilizing specific dibasic acids which meet the foregoing requirements.

### DETAILED DESCRIPTION OF THE INVENTION

First, the compound of formula I used in the invention is described.

In formula I, L represents a linear or branched alkylene group having 1 to 10 carbon atoms, preferably 1 to 5 carbon atoms, which may have a substituent. Preferable examples thereof include a methylene, ethylene, trimethylene and propylene group. Examples of the substituent include a carboxyl group, sulfo group, phosphono group, phosphinic acid group, hydroxyl group, ammonio group which may have an alkyl substituent; among them, a carboxyl group, sulfo group, phosphono group and hydroxyl group are preferred. A represents a carboxyl group, sulfo group, phosphono group, phosphinic acid group, hydroxyl group, amino group which may have an alkyl substituent, ammonio group which may have an alkyl substituent, carbamoyl group which may have an alkyl substituent, sulfamoyl group which may have an alkyl substituent; preferred among them are a carboxyl group, sulfo group, hydroxyl group, phosphono group and carbamoyl group which may have an alkyl substituent. Preferred examples of -L-A- include a carboxymethyl, carboxyethyl, carboxypropyl, sulfoethyl, sulfopropyl, sulfobutyl, phosphonomethyl, phosphonoethyl and hydroxyethyl group; particularly preferred are a carboxymethyl, carboxyethyl, sulfoethyl, sulfopropyl, phosphonomethyl and phosphonoethyl group. R represents a hydrogen atom or a linear or branched alkyl group having 1 to 10 carbon atoms, preferably 1 to 5 carbon atoms, which may have a substituent. Examples of the substituent include a carboxyl group, sulfo group, phosphono group, phosphinic acid group, hydroxyl group, amino group which may have an alkyl substituent, ammonio group which may have an alkyl substituent, carbamoyl group which may have an alkyl substituent and sulfamoyl group which may have an alkyl substituent. Two or more substituents may be present. Preferred examples of R include a hydrogen atom and a carboxymethyl, carboxyethyl, carboxypropyl, sulfoethyl, sulfopropyl, sulfobutyl, phosphonomethyl, phosphonoethyl and hydroxyethyl group; among them, a hydrogen atom and a carboxymethyl, carboxyethyl, sulfoethyl, sulfopropyl, phosphonomethyl and phosphonoethyl group are particularly preferred. L and R may link with each other to form a ring.

Typical examples of the compound represented by formula I are shown below.

(19) HO-NH-CH₂CO₂H

(28) HO-NH-(CH₂)₃SO₃H

(29) HO-NH-(CH₂)₄SO₃H

(32) HO-NH-CH₂CH₂PO₃H₂

(33) HO-NH-CH₂CH₂OH

(34) HO-NH-(CH₂)₃OH

(35) HO-NH-CH₂-PO₃H₂

These compounds are contained in a color developer in an amount of 1.5 × 10⁻³ to 1.5 × 10⁻¹ mol, preferably 3.0 × 10⁻³ to 9.0 × 10⁻² mol, per liter of color developer.

These compounds may be further contained in a light-sensitive material. Further, when contained in a processing solution other than color developer, such as a bleach, bleach-fixer, rinsing solution or stabilizer as substitute for rinsing solution, these compounds act upon color developing agents or oxidation products thereof brought into these solutions from a color developer and provide a light-sensitive material with preferable photographic properties.

The compounds represented by formula I can be synthesized by alkylation (nucleophilic displacement reactions, addition reactions or Mannich reactions) of hydroxylamines available on the market. Useful synthesis methods can be seen in German Pat. No. 1,159,634 and Inorganica Chimica Acta, Vol. 93 (1984), pp. 101-107.

The term "monosaccharide" used in the invention is a general name for polyhydroxyaldehydes, polyhydroxyketones and a broad range of their derivatives including their reduction derivatives, oxidation derivatives, deoxy-derivatives, amino-derivatives and thio-derivatives. In the invention, saccharides represented by formula CₙH₂ₙOₙ as well as compounds derived from the saccharide skeleton represented by this formula are defined as monosaccharides. Among these monosaccharides, preferred are ones having 3 to 7 carbon atoms, such as trioses, tetroses, pentoses, hexoses, heptoses and derivatives thereof.

Typical exemplified compounds of the monosaccharides used in the invention are as follows:
Exemplified Compounds
(1) Glyceraldehyde
(2) Dihydroxyacetone (including dimer)
(3) D-Erythrose
(4) L-Erythrose
(5) D-Threose
(6) L-Threose
(7) D-Ribose
(8) L-Ribose
(9) D-Arabinose
(10) L-Arabinose
(11) D-Xylose
(12) L-Xylose
(13) D-Lyxose
(14) L-Lyxose
(15) D-Xylulose
(16) L-Xylulose
(17) D-Ribulose
(18) L-Ribulose
(19) 2-Deoxy-D-ribose
(20) D-Allose
(21) L-Allose
(22) D-Altrose
(23) L-Altrose
(24) D-Glucose
(25) L-Glucose
(26) D-Mannose
(27) L-Mannose
(28) D-Gulose
(29) L-Gulose
(30) D-Idose
(31) L-Idose
(32) D-Galactose
(33) L-Galactose
(34) D-Talose
(35) L-Talose
(36) D-Quinovose
(37) Digitalose
(38) Digitoxose
(39) Cymarose
(40) D-Sorbose
(41) L-Sorbose
(42) D-Tagatose
(43) D-Fucose
(44) L-Fucose
(45) 2-Deoxy-D-glucose
(46) D-Psicose
(47) D-Fructose
(48) L-Fructose
(49) L-Rhamnose
(50) D-Glucosamine
(51) D-Galactosamine
(52) D-Mannosamine
(53) D-Glycero-D-galactoheptose
(54) D-Glycero-D-mannoheptose
(55) D-Glycero-L-mannoheptose
(56) D-Glycero-D-guloheptose
(57) D-Glycero-D-idoheptose
(58) D-Glycero-L-glucoheptose
(59) D-Glycero-L-taloheptose
(60) D-Altroheptulose
(61) D-Mannoheptulose
(62) D-Altro-3-heptulose
(63) D-Glucuronic acid
(64) L-Glucuronic acid
(65) N-Acetyl-D-glucosamine

Among these exemplified compounds, preferred are those shown by (1), (7), (8), (9), (10), (11), (12), (17), (19), (20), (24), (25), (26), (27), (32), (33), (40), (41), (47), (48), (50), (63) and (65); those denoted by (1), (7), (8), (40), (41), (47), (48) and (50) are particularly preferred.

In the embodiment of the invention, the addition amount of the monosaccharides is 1.5 × 10⁻³ to 1.5 × 10⁻¹ mol, preferably 3.0 × 10⁻³ to 9.0 × 10⁻² mol and especially 4.5 × 10⁻³ to 6.0 × 10⁻² mol per liter of color developer.

In the invention, it is preferred that the color developer contains an aromatic compound having a sulfonic acid group or an aromatic compound having a sulfate group represented by the following formula II or III.

In the formula, A to F are each independently -SO₃M, -OSO₃M, a hydrogen atom, a halogen atom or a saturated or unsaturated hydrocarbon group provided that at least one of the groups represented by A to F is -SO₃M group, M is a hydrogen atom, an alkali metal atom or an ammonium group.

In the formula, G to N are each independently -SO₃M, -OSO₃M, a hydrogen atom, a halogen atom, an alkyl group, an alkenyl group or an alkynyl group, M is a hydrogen atom, an alkali metal atom or an ammonium group.

In formula II or III, the alkyl, ankenyl or alkynyl group represented by A to F or G to N is preferably one having 1 to 10 carbon atoms. Its carbon chain may be either linear or branched.

Typical examples of the compounds represented by formula II or III are shown below, but the scope of the invention is not limited to them. Though these exemplified compounds are shown in the form of sodium salts, these sodium salts may be wholly or partly -SO₃H or -OSO₃H.

| Exemplified compounds No. | G | H | I | J | K | L | M | N |
|---|---|---|---|---|---|---|---|---|
| III-1 | -SO₃Na | H | H | H | H | H | H | H |
| III-2 | H | -SO₃Na | H | H | H | H | H | H |
| III-3 | H | -SO₃Na | H | H | H | -CH₃ | H | H |
| III-4 | -SO₃Na | H | H | H | -SO₃Na | H | H | H |
| III-5 | H | -SO₃Na | H | H | H | -SO₃Na | H | H |
| III-6 | H | H | -SO₃Na | H | H | -SO₃Na | H | H |
| III-7 | H | -SO₃Na | H | -SO₃Na | H | H | H | H |
| III-8 | -SO₃Na | H | -SO₃Na | H | H | -SO₃Na | H | H |
| III-9 | -CH₃ | H | -SO₃Na | H | H | -SO₃Na | H | H |
| III-10 | -Cl | H | -SO₃Na | H | H | -SO₃Na | H | H |
| III-11 | H | -SO₃Na | H | H | H | -SO₃Na | H | -Cl |
| III-12 | H | H | -SO₃Na | H | H | -Cl | H | H |
| III-13 | H | H | -O-SO₃Na | H | H | -O-SO₃Na | H | H |
| III-14 | -O-SO₃Na | H | -O-SO₃Na | H | H | -O-SO₃Na | H | H |

The addition amount of the compounds represented by formula II or III is preferably not less than 5 g/l, more preferably in the range of 10 to 200 g/l.

In the invention, conventional P-phenylenediamine color developing agents can be used. Preferred color developing agents are those exemplified as follows. Concerning color developing agents Japanese Pat. O.P.I. Publication No. 86741/1992 may be referred. In the following, color developing agent (C-1) can bring out the effect of the invention most pronouncedly.

Preferably, these color developing agents are used in the form of hydrochlorides, sulfates, nitrates or p-toluenesulfonates.

In the invention, the color developing agents are used within the range of 2.5 × 10⁻³ to 5.5 × 10⁻² mol, preferably 5.0 × 10⁻³ to 4.5 × 10⁻² mol per liter of color developer.

In addition to the above components, the color developer used in the invention may contain the following components usually used in color developer.

As alkali agents, there may be used, singly or in combination, sodium hydroxide, potassium hydroxide, silicates, sodium metaborate, potassium metaborate, trisodium phosphate, tripotassium phosphate and borax within a range necessary to maintain the pH stabilizing effect without forming precipitates. Further, for the sake of compounding or for the purpose of raising ion intensity, there may be used a variety of salts including disodium hydrogenphosphate, dipotassium hydrogenphosphate, sodium bicarbonate, potassium bicarbonate and borates.

Preferably, the color developing replenisher used in the invention contains an optical whitening agent. Using an optical whitening agent not only improves the whiteness of light-sensitive materials' nonexposed portions, but also prevents crystals from depositing.

Triazinylstilbene optical whitening agents are preferred in the invention, particularly preferred are those represented by the following formula F.

In Formula F, X₁, X₂, Y₁ and Y₂ are each a hydroxyl group, halogen atom such as chlorine and bromine, an alkyl group such as a methyl group and an ethyl group, an aryl group such as a phenyl group and a methoxyphenyl group, a group, a group or a -OR₂₅ group, In the above, R₂₁ and R₂₂ are each a hydrogen atom, an alkyl group which may have a substituent, or a aryl group which may have a substituent; R₂₃ and R₂₄ are each an alkylene group which may have a substituent; R₂₅ is a hydrogen atom, an alkyl group or an aryl group, they may have a substituent; M is a cation such as sodium, potassium, lithium or ammonium. An alkyl group represented by R₂₁, R₂₂ or R₂₅ are preferably one having 1 to 6 carbon atoms, and an alkylene group represented R₂₃ or R₂₄ are preferably one having 1 to 2 carbon atoms.

A group which may be a substituent of an alkyl group or an aryl group represented by R₂₁, R₂₂ or R₂₅, or an alkylene group represented by R₂₃ or R₂₄ is preferably a hydroxyl group, a sulfo group, or a carboxylamino group.

As group represented by the following groups are exemplified; am amino group, an alkylamino group such as a methylamino group, ethylamino group, propylamino group, dimethylamino group, cyclohexylamino group, β-hydroxyethylamino group, di(β-hydroxyethyl)amino group, β-sulfoethylamino group, N-(β-sulfoethyl)-N-methylamino group and N-(β-hydroxyethyl)-N-methylamino group; and an arylamino group such as an anilino group, o-sulfoanilino group, m-sulfoanilino group, p-sulfoanilino group, o-chloroanilino group, m-chloroanilino group, p-chloroanilino group, o-toluidino group, m-toluidino group, p-toluidino group, o-carboxyanilino group, m-carboxyanilino group, p-carboxyanilino group, o-hydroxyanilino group, m-hydroxy-anilino group, p-hydroxyanilino group, sulfonaphthylamino group, o-aminoanilino grop, m-aminoanilino grop, p-amino-anilino grop, o-anidino group, m-anidino group, m-anidino group. As an example of groups represented by a morpholino group is cited. As groups represented by -OR₂₅, an alkoxy group such as a methoxy group, ethoxy group and methoxyethoxy group, and an aryloxy group such as a phenoxy group and p-sulfophenoxy group, are exemplified.

Among optical whitening agents represented by Formula F, preferable compounds are ones in which all groups represented by X₁, X₂, Y₁ and Y₂ are a group represented by or -OR₂₅, and most preferable compounds are ones in which one of X₁ and Y₁ is -OR₂₅ and the other is a group represented by and one of X₂ and Y₂ is -OR₂₅ and the other is a group represented by or

Typical examples of the compounds represented by formula F include compounds the following F-1 to F-7. Concerning the optical whitening agents Japanese Pat. Appl. No. 178833/1990 can be referred. These triazinylstilbene optical whitening agents can be synthesized by the usual method described, for example, in "Optical Whitening Agents", edited by Kaseihin Kogyo Kyokai (Aug., 1976), p. 8.

The triazinylstilbene optical whitening agents are used in amounts of preferably 0.2 to 10 g, especially 0.4 to 5 g, per liter of color developing replenisher. Further, in order to enhance the effect of the invention much more, it is preferred that the chelating agent of the following formula K be added to the color developing replenisher.

In Formula K, E is a substituted or unsubstituted alkylene group, a cycloalkylene group, a phenylene group, a -R₅OR₅- group, a -R₅OR₅OR₅- group or a -R₅ZR₅- group; Z is a >N-R₅-A₅ group or a >N-A₅ group; R₁ to R₅ are each a substituted or unsubstituted alkylene group; A₁ to A₅ are each a hydrogen atom, a -OH group, a -COOM group or a -PO₃(M)₂ group; and M is a hydrogen atom or an alkali metal atom. Typical example of the compounds represented by Formula K include the following compounds K-1 to K-22.

In the invention, the pH of the color developer is preferably in the range of 9.5 to 13.0, more preferably in the range of 9.8 to 12.5.

In the invention, when the color developing time is in the range of 35 to 55 seconds, the replenishing rate of the color developer is not more than 120 ml/m², preferably 20 to 100 ml/m². When the color developing time is in the range of 5 to 30 seconds, the replenishing rate, though it depends upon the color developing time, is in the range of 50 to 200 ml/m².

Next the aliphatic dibasic acid used in the invention is described. The aliphatic dibasic acid used in the invention undergoes a chelate exchange reaction more effectively than other acids in the coating layer of a light-sensitive material; therefore, it retards the chelate exchange reaction of aminopolycarboxylic acids and effectively prevents desilverizing failure and recoloring failure.

The aliphatic dibasic acid used in the invention is selected from oxalic acid, succinic acid, maleic acid, fumaric acid and adipic acid.

These aliphatic dibasic acids are added to the bleach-fixer in amounts of 1.5 × 10⁻² to 8.5 × 10⁻¹ mol, preferably 8.0 × 10⁻² to 4.3 × 10⁻¹ mol per liter of bleach-fixer.

Aminopolycarboxylic acid complex salts used in the invention include ethylenediaminetetraacetic acid ferric complex salts, diethylenetriaminepentaacetic acid ferric complex salts, trans-1,2-cyclohexanediaminetetraacetic acid ferric complex salts, β-alaninediacetic acid ferric complex salts, ethylenediaminedisuccinic acid ferric complex salts, nitrilotriacetic acid ferric complex salts, N-hydroxyethylethylenediaminetriacetic acid ferric complex salts and glycol ether-diaminetetraacetic acid ferric complex salts.

The aminopolycarboxylic acid ferric complex salts are used in an amount of not less than 0.01 mol per liter of bleach-fixer, preferably within the range of 0.03 to 0.3 mol/l and especially within the range of 0.05 to 0.25 mol/l.

As fixing agents contained in the bleach-fixer of the invention, conventional ones can be used. Preferred are thiocyanates and thiosulfates.

The addition amount of the fixing agents is preferably not less than 0.1 mol /l, more preferably 0.3 to 4 mol/l, even more preferably 0.5 to 3 mol/l, and most preferably 0.6 to 2.0 mol/l.

For the purposes of enhancing the effect of the invention and achieving an ammonia-free processing, it is preferred that the bleach-fixer contain the compound of formula FA or compound included in Group FB.

Further, it is also preferred that the sulfurous acid adducts represented by formula A-I or A-II.

In formula FA, R' and R'' are each a hydrogen atom, an alkyl group, an aryl group, an aralkyl group or a nitrogen-containing heterocyclic group; and n' is an integer of 2 or 3.

Typical example of the compounds represented by Formula FA are as follows.

These compounds represented by Formula FA can be synthesized by ordinary synthesis methods such described as in US Patents Nos. 3,335,161 and 3,260,718.

Group of compounds FB
- FB-1: Thiourea
- FB-2: Ammonium iodide
- FB-3: Potassium iodide
- FB-4: Ammonium thiocyanate
- FB-5: Potassium thiocyanate
- FB-6: Sodium thiocyanate
- FB-7: Thicyanocatechol

In the above Formulas A-I and A-II, A₂, A₃, A₄ and A₅ are each a hydrogen atom, an alkyl group having 1 to 6 carbon atoms, a formyl group, an acyl group or an alkenyl group. The alkyl groups having 1 to 6 carbon atoms including ones having straight chain and ones having a branched chain, include, for example, a methyl group, ethyl group, n-propyl group, isopropyl group, n-butyl group, n-pentyl group, iso-pentyl group, n-hexyl group or iso-hexyl group. The alkyl group may have a substituent. The substituted alkyl groups include ones having formyl group such as formyl methyl group and 2-formylethyl group, ones having amino group such as aminomethyl group and aminoethyl group, ones having hydroxyl group such as hydroxymethyl group, 2-hydroxyethyl group and 2-hydroxypropyl group, alkoxy group such as methoxy group and ethoxy group, ones having halogen atom such as chloromethyl group, trichlorometyl group and dibromomethyl group.

The alkenyl group may have a substituent. Unsubstituted alkenyl groups include, for example, vinyl group and 2-propenyl group, and substituted alkenyl groups include, for example, 1.2-dichlorocarboxyvinyl group and 2-phenylvinyl group.

Silver may be recovered by a conventional method from the bleach-fixer according to the invention. In addition to these fixing agents, the bleach-fixer may contain, singly or in combination, sulfites and pH buffers selected from a variety of salts. Further, rehalogenating agents including alkali halides and ammonium halides, such as potassium bromide, sodium bromide, sodium chloride and ammonium bromide, are preferably added thereto in large quantities. Moreover, compounds such as alkylamines and polyethylene oxides, which are known to be added to a bleach-fixer, may also be added.

The bleach-fixer is used in the pH range of preferably 1.0 to 8.5, more preferably 1.5 to 8.0.

When the bleach-fixing time ranges from 35 to 55 seconds in embodying the invention, the replenishing rate is 30 ml/m² to 120 ml/m² of light-sensitive material process, preferably 40 ml/m² to 100 ml/m². When the bleach-fixing time is in the range of 5 to 30 seconds, the replenishing rate is 50 to 250 ml/m².

In a preferred embodiment of the invention, the process using a fixing-capable processing solution is followed by a stabilizing process without performing a substantial washing process.

Preferably, the stabilizer used in the stabilizing process contains the chelating agent of formula CH-I, CH-II or CH-III.

In the above formula, E is an alkylene group, a cycloalkylene group, a phenylene group, a -R₅'-O-R₅'- group, a -R₅'-O-R₅'-O-R₅'- group, or -R₅'-Z-R₅'- group. Z is a >N-R₅'-A₅ group, a group, a >N-A₅ group or a group. R₁' to R₆' are each an alkylene group, and A₁ to A₃ are each a -COOM group or a -PO₃M₂ group and A₄ and A₅ are each a hydrogen atom, a hydroxyl group, a -COOM group or a -PO₃M₂ group. M is a hydrogen atom or an alkali metal atom.

In the above, R₇' is an alkyl group, an aryl group or a nitrogen-containing six-member ring, M is a hydrogen atom or an alkali metal atom.

In the above, R₈', R₉' and R₁₀' are each a hydrogen atom, a hydroxyl group, a -COOM group, a -PO₃M₂ group or a group, in which J is a hydrogen atom, an alkyl group, a -C₂H₄OH group or a -PO₃M₂ group; M is a hydrogen atom or an alkali metal atom; and n and m are each 0 or 1.

Examples of compounds represented by Formula CH-I, CH-II or CH-III are given in the followings.

The addition amount of the chelating agent is preferably 0.01 to 100 g, more preferably 0.05 to 50 g, and most preferably 0.1 to 20 g per liter of stabilizer. It is also preferred that metal salts be contained in the stabilizer together with the chelating agent. Examples of such metal salts include salts of Ba, Ca, Ce, Co, In, La, Mn, Ni, Bi, Pb, Sn, Zn, Ti, Zr, Mg, Al and Sr. These can be fed as inorganic salts including halides, hydroxides, sulfates, carbonates, and phosphates or as water-soluble chelated compounds.

Further, the stabilizer may contain organic acids such as citric acid, acetic acid, succinic acid, oxalic acid, benzoic acid and pH adjustors such as phosphates, borates, hydrochlorides, sulfates.

In the invention, conventional fungicides can be contained singly or in combination in the stabilizer within the range not harmful to the effect of the invention. Silver may be recovered from the stabilizer according to the usual method. Further, the stabilizer may be subjected to ion exchange treatment, electrodialysis (see Japanese Pat. O.P.I. Pub. No. 28949/1986) or reverse osmosis (see Japanese Pat. O.P.I. Pub. Nos. 240153/1985 and 254151/1987), or the water used in the stabilizer may be deionized in advance, in order to enhance the fungus resistance and stability of the stabilizer as well as image preservability. Any deionizing method can be used as long as it can reduce the content of calcium and magnesium ions in the water after treatment to 5 ppm or less; but, treatments with ion exchange resins or reverse osmosis membranes, or combinations thereof, are preferred. Details of ion exchange resins and reverse osmosis membranes can be seen in Journal of Technical Disclosure Nos. 1984/1987 and 20511/1989.

No washing is required after the stabilizing process. But, if necessary, an extremely short-time rinsing or surface washing with a small amount of water may be carried out.

In the embodiment of the invention, the stabilizer pH is preferably in the range of 5.5 to 10.0. Any of the conventional alkali agents and acid agents can be used as a pH adjustor for the stabilizer.

The stabilizing process is carried out at temperatures of preferably 15 to 70°C, more preferably 20 to 55°C. The stabilizing time is usually not longer than 120 seconds, preferably 3 to 90 seconds and most preferably 6 to 50 seconds.

The replenishing volume of the stabilizer per unit area of light-sensitive material is preferably 0.1 to 80 times, more preferably 0.5 to 30 times the volume of the preceding solution, fixer or bleach-fixer, brought into the stabilizing bath, in view of rapid processability and dye image preservability.

It is desirable that the stabilizing tank be made up of plural tanks, preferably 2 to 6 tanks. In a particularly preferred mode, two or three tanks are arranged countercurrently and the stabilizer is fed to the rear tank and overflowed from the front tank.

Next, the color light-sensitive material suitable for the invention is described.

As silver halide grains used in the light-sensitive material, silver chloride rich silver halide grains having a silver chloride content of 80 mol% or more are employed. The silver chloride content of these grains is preferably not less than 90 mol%, more preferably not less than 95 mol%, and most preferably not less than 98 mol%.

Silver halide emulsions comprising the above silver chloride rich silver halide grains may contain, as silver halide components, silver bromide and/or silver iodide besides silver chloride. In this case, the content of silver bromide is preferably not more than 10 mol%, more preferably not more than 5 mol%, and most preferably not more than 2 mol%. When silver iodide is contained, its content is preferably not more than 1 mol%, more preferably not more than 0.5 mol%, and most preferably zero. Such silver chloride rich silver halide grains containing 90 mol% or more silver chloride will work when used at least in one silver halide emulsion layer; but, preferably, these are used in all light-sensitive silver halide emulsion layers.

The above silver halide grains may be regular crystals, twin crystals or other crystal forms, and these may have any [1.0.0] face to [1.1.1] face ratio. The crystal structure of these grains may be uniform from the inner portion to the outer portion or may be the core/shell structure that comprises inner and outer layers having phases different in composition. Further, these grains may be those which form latent images mainly on the surface or those which form latent images mainly inside of the grains. There may also be used tabular silver halide grains disclosed, for example, in Japanese Pat. O.P.I. Pub. No. 113934/1983 and No. 47959/1986 as well as the silver halides disclosed in Japanese Pat. O.P.I. Pub. Nos. 26837/1989, 26838/1989, 77047/1989.

These silver halide grains may be prepared by any of the acid method, the neutral method and the ammoniacal method.

These methods may also be combined. In a preferable combination, seed grains are formed by the acid and, then, grown to a prescribed size by the ammoniacal method which can give a faster growth rate.

In growing the silver halide grains, it it preferred that silver ions and halide ions be simultaneously introduced in amounts corresponding to the growth rate of silver halide grains as described, for example, in Japanese Pat. O.P.I. Pub. No. 48521/1979 with the pH and pAg of the reaction system being controlled.

Silver halide emulsion layers of the light-sensitive material to be processed according to the invention contain color couplers.

The red-sensitive emulsion layer may contain, for example, nondiffusible color couplers to form cyan portion color images, namely, phenol-type or α-naphthol-type couplers in general.

The green-sensitive emulsion layer may contain, for example, at least one nondiffusible color coupler to form magenta portion color images, namely, 5-pyrazolone-type or pyrazolotriazole-type color couplers in general. The blue-sensitive emulsion layer may contain, for example, at least one nondiffusible color coupler to form yellow portion color images, namely, color couplers having an open-chain ketomethylene group in general. These color couplers may be 6-, 4- or 2-equivalent couplers.

In the invention, particularly preferred are the 2-equivalent couplers.

Suitable couplers can be seen, for example, in W. Pelz, Farbkuppler (Color Couplers) contained in Mitteilungen aus den Forschungslaboratorien der Agfa (Research Papers of Agfa), Leverkusen/Munchen, Vol. III, p. 111 (1961); K. Venkataraman, The Chemistry of Synthetic Dyes, Vol. 4, pp. 341-387, Academic Press; The Theory of the Photographic Process, 4th edition, pp. 353-362; and Research Disclosure No. 17643, Sec. VII.

In view of the effect of the invention, particularly preferred couplers are the magenta couplers represented by formula M-1 on page 26 of Japanese Pat. O.P.I. Pub. No. 106655/1988, typical examples thereof are magenta coupler Nos 1 to 77 shown on pages 29-34 of the same patent specification; the cyan couplers represented by formula C-1 or C-II on page 34 of the same specification, typical examples thereof are cyan couplers C'-1 to C'-82 and C"-1 to C"-36 shown on pages 37-42 of the same specification; and the rapid reactive yellow couplers described on page 20 of the same specification typical examples thereof are yellow couplers Y'-1 to Y'-39 shown on pages 21-26 of the same specification.

When nitrogen-containing heterocyclic mercapto compounds are used in a light-sensitive material comprising a silver chloride rich emulsion, not only is the effect of the invention well enhanced, but undesired influences on photographic properties caused by the contamination of a color developer with a bleach-fixer can be effectively diminished. Accordingly, use of these compounds is preferred in the embodiment of the invention.

Typical examples of such nitrogen-containing heterocyclic mercapto compounds include compounds I'-1 to I'-87 exemplified on pages 42-45 of Japanese Pat. O.P.I. Pub. No. 106655/1988.

The silver halide emulsion can be prepared by the usual method, for example, constant rate or accelerated rate single-jet or double-jet pouring of the materials. Particularly preferred is the double-jet under a controlled pAg (see Research Disclosure No. 17643, Secs. I and II).

The silver halide emulsion can be chemically sensitized. Sulfur-containing compounds such as allyl isothiocyanate, allyl thiourea and thiosulfates are particularly preferred chemical sensitizers. Reducing agents can also be employed as chemical sensitizers; examples thereof include silver compounds as disclosed in Belgian Pat. Nos. 493,464, 568,687 as well as polyamines such as diethylenetriamine and aminodimethylsulfinic acid derivatives as disclosed in Belgian Pat. No. 547,323. Other suitable sensitizers are noble metals, such as gold, platinum, palladium, iridium, ruthenium, rhodium, and compounds thereof. Such chemical sensitization is described in detail in R. Kosiovsky's monograph contained in Z. Wiss. Photo., Vol. 46, pp. 65-72 (1951) (see also Research Disclosure No. 17643, Sec. III).

The silver chloride rich emulsion can be optically sensitized by conventional methods including those which employ ordinary polymethine dyes such as neutro-cyanine, basic or acid carbocyanine, rhodacyanine, hemicyanine; styryl dyes, oxonol and its analogues. Details of optical sensitization can be seen in F.M. Hamer, The Cyanine Dyes and Related Compounds (1964), Ullmanns Enzyklpadie der Technischen Chimi, 4th Edition, Vol. 18, p. 431 and Research Disclosure No. 17643, Sec. IV.

The silver chloride rich emulsion can use conventional antifoggants and stabilizers. Azaindenes are useful stabilizers, preferred are tetra- and penta-azaindene, and particularly preferred are those substituted with a hydroxyl group or amino group. These compounds are described, for example, in Birr's monograph contained in Z. Wiss. Photo., Vol. 47 (1952), pp. 2-58 and Research Disclosure No. 17643, Sec. IV.

The component of the light-sensitive material can be incorporated by conventional methods as described, for example, in U.S. Pat. Nos. 2,322,027, 2,533,514, 3,689,271, 3,764,336, 365,897. The components such as couplers and UV absorbents can be incorporated in the form of charged latex as described, for example, in German Offenlegungshrift No. 2,541,274 and European Pat. Appl. No. 14,921. Further, the component can be set in the form of polymer in a light-sensitive material as described, for example, in German Offenlegungshrift No. 2,044,992 and U.S. Pat. Nos. 3,370,952, 4,080,211.

As supports for the color photographic light-sensitive material to be processed according to the invention, there can be used baryta paper; polyethylene-coated paper; polypropylene synthetic paper; transparent supports having a reflective layer or functioning as a reflective body, such as glass plates, films of polyesters including cellulose acetate, cellulose nitrate, polyethylene terephthalate, polyamide films, polycarbonate films, polystyrene films; and other conventional transparent supports. These supports are properly selected according to the end use of light-sensitive materials. But, in order to achieve the object of the invention effectively, reflective supports such as baryta paper, polyethylene-coated paper and polypropylene synthetic paper are preferred.

The invention can be applied to color light-sensitive materials such as color paper, color negative films, color reversal films, color reversal paper and direct positive color paper for popular uses or for movies as well as color films for movies and color films for television.

The processing method of the invention is applicable to any automatic processor, but the effect of the invention can be most enhanced by use of an automatic processor whose opening area, per liter surface area of a processing solution, is not larger than 12 cm²/l, preferably not larger than 10 cm²/l.

### EXAMPLES

### Example 1

### Preparation of Silver Halide Color Photographic Light-sensitive Material (Color Paper)

A multilayered silver halide color photographic light-sensitive material was prepared by forming the layers shown in Tables 1 and 2 on a paper support laminated with polyethylene on one side and with titanium-oxide-containing polyethylene on the other side to be coated with the above component layers.

The coating solutions were prepared as follows:

### Coating Solution for 1st Layer

In 6.67 g of high boiling solvent (DNP) and 60 ml of ethyl acetate were dissolved 26.7 g of yellow coupler Y-1, 100 g of dye image stabilizer ST-1, 6.67 g of dye image stabilizer ST-2 and 0.67 g of additive HQ-1. The solution was then dispersed with an ultrasonic homogenizer in 220 ml of 10% aqueous gelatin solution containing 7 ml of 20% surfactant SU-1 to obtain a yellow coupler dispersion. This dispersion was mixed with a blue-sensitive silver halide emulsion containing 10 g of silver prepared under the following conditions to obtain a coating solution for 1st layer.

Coating solutions for the 2nd to 7th layers were prepared likewise. As hardeners, hardener H-1 was added to the 2nd layer and the 4th layer and hardener H-2 to the 7th layer. As coating aids, surfactants SU-2 and SU-3 were added to adjust the surface tension.

Structural formulas of the compounds used in the above light-sensitive material are as follows:
- DOP :: dioctyl phthalate
- DNO :: dinonylphenol
- DIDP:: diisodecyl phthalate
- PVP :: polyvinylpyrrolidone

### Preparation of Blue-sensitive Silver Halide Emulsion

The following solutions A and B were simultaneously added to 1000 ml of 2% aqueous gelatin solution kept at 40°C in 30 minutes, with the pAg and pH controlled at 6.5 and 3.0, respectively. Then, the following solutions C and D were simultaneously added thereto in 180 minutes with the pAg and pH controlled at 7.3 and 5.5, respectively.

In the cause of preparation of the emulsion the pH was controlled by use of sulfuric acid or an aqueous solution of sodium hydroxide.

The control of the pAg was carried out by use of a controlling solution, which was an aqueous solution of a halide salt mixture comprising sodium chloride and potassium bromide with a chloride ion-to-bromide ion ratio of 99.8:0.2. It was used at a concentration of 0.1 mol/l while solutions A and B were added, and at a concentration of 1 mol/l while solutions C and D were added.

### Solution A

| | |
|---|---|
| Sodium chloride | 3.42 g |
| Potassium bromide | 0.03 g |
| Water was added to | 200 ml |

### Solution B

| | |
|---|---|
| Silver nitrate | 10 g |
| Water was added to | 200 ml |

### Solution C

| | |
|---|---|
| Sodium chloride | 102.7 g |
| Potassium bromide | 1.0 g |
| Water was added to | 600 ml |

### Solution D

| | |
|---|---|
| Silver nitrate | 300 g |
| Water was added to | 600 ml |

After completing the addition, the resulting silver halide emulsion were desalted with 5% aqueous solution of Demol N made by Kao-Atlas Co. and 20% aqueous solution of magnesium sulfate and, then, mixed with an aqueous solution of gelatin. Emulsion EMP-1 so-prepared comprised monodispersed cubic grains having an average grain size of 0.85 µm, a coefficient of variation of grain size distribution of 7% and a silver chloride content of 99.5 mol%.

Subsequently, Emulsion EMP-1 was chemically ripened for 90 minutes at 50°C, using the following compounds, to obtain a blue-sensitive silver halide emulsion (Em-A).

| | |
|---|---|
| Sodium thiosulfate | 0.8 mg/mol AgX |
| Chloroauric acid | 0.5 mg/mol AgX |
| Stabilizer STAB-1 | 6 × 10⁻⁴ mol/mol AgX |
| Sensitizing dye BS-1 | 4 × 10⁻⁴ mol/mol AgX |
| Sensitizing dye BS-2 | 1 × 10⁻⁴ mol/mol AgX |

### Preparation of Green-sensitive Silver Halide Emulsion

The procedure of emulsion EMP-1 was repeated except that the addition time of solutions A and B and that of solutions C and D were changed. Emulsion EMP-2 so-prepared comprised monodispersed cubic grains having an average grain size of 0.43 µm, a coefficient of variation of grain size distribution of 8%, and a silver chloride content of 99.5 mol%.

Emulsion EMP-2 was chemically ripened for 120 minutes at 55°C, using the following compounds, to obtain a green-sensitive silver halide emulsion (Em-B).

| | |
|---|---|
| Sodium thiosulfate | 1.5 mg/mol AgX |
| Chloroauric acid | 1.0 mg/mol AgX |
| Stabilizer STAB-1 | 6 × 10⁻⁴ mol/mol AgX |
| Sensitizing dye GS-1 | 4 × 10⁻⁴ mol/mol AgX |

### Preparation of Red-sensitive Silver Halide Emulsion

The procedure of emulsion EMP-1 was repeated except that the addition time of solutions A and B and that of solutions C and D were changed. Emulsion EMP-3 so-prepared comprised monodispersed cubic grains having an average grain size of 0.50 µm, a coefficient of variation of grain size distribution of 8%, and a silver chloride content of 99.5 mol%.

Emulsion EMP-3 was chemically ripened for 90 minutes at 60°C, using the following compounds, to obtain a red-sensitive silver halide emulsion (Em-C).

| | |
|---|---|
| Sodium thiosulfate | 1.8 mg/mol Agx |
| Chloroauric acid | 2.0 mg/mol Agx |
| Stabilizer STAB-1 | 6 × 10⁻⁴ mol/mol Agx |
| Sensitizing dye RS-1 | 4 × 10⁻⁴ mol/mol Agx |

The following are the structural formulas of the compounds used in the preparation of the above emulsions.

The silver chloride content of the color paper sample prepared as above was 99.5 mol%. Color paper samples 1 to 23 were prepared by varying the silver chloride content as shown in Table 3.

The samples were wedgewise exposed by the usual method and then subjected to continuous processing in accordance with the following process (1):

| Process (1) | Processing Temp. (°C) | Processing Time (sec.) | Replenishing Rate (ml/m²) |
|---|---|---|---|
| Color developing | 38.5 | 45 | 80 |
| Bleach-fixing | 35 - 37 | 45 | 54 |
| Stabilizing* | 30 - 37 | 30 × 3 | 180 |
| Drying | 60 - 80 | 30 | - |

| | | | |
|---|---|---|---|
| * A 3-tank countercurrent mode, in which the replenisher was poured into the 3rd tank. | | | |

### Color Developing Tank Solution and Replenisher

### Bleach-fixing Tank Solution and Replenisher

| | Tank Solution | Replenisher |
|---|---|---|
| Frric complex of aminopolycarboxylic acid (show in table 3) | 0.15 mol | 0.30 mol |
| Ethylenediaminetetraacetic acid | 2.0 g | 2.0 g |
| Ammonium thiosulfate | 75.0 g | 150 g |
| Ammonium sulfite | 45.0 g | 90.0 g |
| Aliphatic acid (shown in Table 3) | 0.13 mol | 0.26 mol |
| Make up with water to | 1.0 l | 1.0 l |
| pH | 5.50 | 5.30 |

### Stabilizing Tank Solution and Replenisher

This continuous processing according to process (1) was run, using an NPS-1411 small automatic processor, by filling the processor with the above tank solutions and then replenishing the replenishers thereto by means of continuous flow pumps.

The continuous processing was carried on, at a processing speed of 0.1 round per day, till the volume of the replenished stabilizer amounted to three times the volume of the developing tank solution. Here 1 round means that the color developer replenisher is replenished up to a volume equal to the capacity of color developing tank. The minimum reflection density (measured by blue-light) and the maximum reflection density (measured by red-light) were measured with color paper samples exposed wedgewise and processed at the beginning of the continuous run, and with samples exposed wedgewise and processed at the end of the continuous run.

Further, the amount of residual silver was determined by the fluorescence X-ray method with samples exposed and processed at the end of the continuous run.

Table 3 shows measured values of the residual silver amount, the following difference in minimum density (ΔB) and the difference in maximum density (ΔR).
ΔB = minimum reflection density (B) at the end of continuous run - minimum reflection density (B) at the beginning of continuous run
ΔR = maximum reflection density (R) at the end of continuous run - maximum reflection density (R) at the beginning of continuous run

It can be understood from the results in Table 3 that a processing method excellent in stain prevention and recoloring property could be established for the first time by the combination according to the invention.

### Example 2

The procedure of Example 1 was repeated, except that the following process (2) was used and that an NPS-808SQA automatic processor made by Konica Corp. was employed in the continuous run. As a result, the same effect as that in Example 1 was observed.

| Process (2) | Processing Temp. (°C) | Processing Time | Replenishing Rate (ml/m²) |
|---|---|---|---|
| Color developing | 38.5 | 25 sec | 116 |
| Bleach-fixing | 35 - 37 | 25 sec | 200 |
| Stabilizing* | 30 - 37 | 25 sec × 3 | 200 |
| Drying | 60 - 80 | 30 sec | - |

| | | | |
|---|---|---|---|
| * A 3-tank countercurrent mode, in which the replenisher was fed to the 3rd tank. | | | |

### Example 3

The procedure of experiment No. 7 in Example 1 was repeated, except that exemplified compound (7) used as additive was changed to equivalent amounts of exemplified compounds (3), (9), (15), (52), (55), glyceraldehyde, L-ribose, D-sorbose and L-fructose. Though the difference in maximum reflection density (ΔR) became slightly larger, the effect observed was much the same as that in Example 1.

### Example 4

The procedure of experiment No. 7 in Example 1 was repeated, except that the combination of ammonium ferric ethylenediaminetetracetate with the aliphatic dibasic acid in the bleach-fixer was changed to equal moles of the following combinations. The evaluation results were the same as those in Example 1, except that the difference in minimum reflection density (ΔB) became slightly larger.

| No. | Aminopolycarboxylic Acid | Aliphatic Dibasic Acid |
|---|---|---|
| 1 | Ammonium ferric β-alaninediacetate | Maleic acid |
| 2 | Ammonium ferric β-alaninediacetate | Oxalic acid |
| 3 | Ammonium ferric β-alaninediacetate | Succinic acid |
| 4 | Ammonium ferric β-alaninediacetate | Adipic acid |
| 5 | Ammonium ferric ethylenediaminedisuccinate | Maleic acid |
| 6 | Ammonium ferric ethylenediaminedisuccinate | Oxalic acid |
| 7 | Ammonium ferric ethylenediaminedisuccinate | Succinic acid |
| 8 | Ammonium ferric ethylenediaminedisuccinate | Adipic acid |
| 9 | Ammonium ferric diethylenetriaminepentacetate | Maleic acid |
| 10 | Ammonium ferric diethylenetriaminepentacetate | Oxalic acid |
| 11 | Ammonium ferric diethylenetriaminepentacetate | Succinic acid |
| 12 | Ammonium ferric diethylenetriaminepentacetate | Adipic acid |

### Example 5

The procedure of experiment No. 7 in Example 1 was repeated, except that the addition amount of exemplified compound (7) as additive was varied as shown in Table 4. The evaluation results are shown in Table 4.

**Table 4**

| Additive, Exemplified Compound (7), Amount Added (mol/l) | Minimum Reflection Density Difference (ΔB) | Maximum Reflection Density Difference (ΔR) | Amount of Residual Silver (g/m²) |
|---|---|---|---|
| 0 | 0.10 | -0.03 | 0.01 |
| 1.0 × 10⁻³ | 0.05 | -0.02 | 0.01 |
| 1.5 × 10⁻³ | 0.03 | -0.01 | 0.01 |
| 2.0 × 10⁻³ | 0.03 | -0.01 | 0.01 |
| 3.0 × 10⁻³ | 0.01 | -0.04 | 0.01 |
| 1.0 × 10⁻² | 0.01 | -0.01 | 0.01 |
| 5.0 × 10⁻² | 0.01 | -0.01 | 0.01 |
| 9.0 × 10⁻² | 0.01 | -0.01 | 0.01 |
| 1.0 × 10⁻¹ | 0.03 | -0.02 | 0.01 |
| 1.5 × 10⁻¹ | 0.03 | -0.02 | 0.01 |
| 2.0 × 10⁻¹ | 0.04 | -0.03 | 0.01 |

As is shown in Table 4, good results were produced when the addition amount of the additive was 1.5 × 10⁻³ to 1.5 × 10⁻¹ mol/l, much better results were obtained when the addition amount was 3.0 × 10⁻³ to 9.0 × 10⁻² mol/l.

### Example 6

The procedure of experiment No. 7 in Example 1 was repeated, except that the addition amount of the aliphatic dibasic acid (maleic acid) was varied as shown in Table 5. The evaluation results are shown in Table 5.

**Table 5**

| Maleic Acid, Amount Added (mol/l) | Minimum Reflection Density Difference (ΔB) | Maximum Reflection Density Difference (ΔR) | Amount of Residual Silver (g/m²) |
|---|---|---|---|
| 0 | 0.04 | -0.10 | 0.01 |
| 1.0 × 10⁻² | 0.03 | -0.05 | 0.01 |
| 1.5 × 10⁻² | 0.02 | -0.03 | 0.01 |
| 5.0 × 10⁻² | 0.03 | -0.03 | 0.01 |
| 8.0 × 10⁻² | 0.01 | -0.01 | 0.01 |
| 2.0 × 10⁻¹ | 0.01 | -0.01 | 0.01 |
| 4.3 × 10⁻¹ | 0.01 | -0.01 | 0.01 |
| 8.5 × 10⁻¹ | 0.02 | -0.02 | 0.01 |
| 1.0 × 10⁻¹ | 0.03 | -0.04 | 0.01 |
| 1.5 × 10⁻¹ | 0.03 | -0.02 | 0.01 |
| 2.0 × 10⁻¹ | 0.04 | -0.03 | 0.01 |

It will be understood from Table 5 that preferred addition amounts of the aliphatic dibasic acid are in the range of 1.5 × 10⁻² to 8.0 × 10⁻¹ mol/l, and that particularly preferred addition amounts are in the range of 8.0 × 10⁻¹ mol/l.

### Example 7

The procedure of experiment No. 7 in Example 1 was repeated, except that the aromatic sulfinic acids were changed to the compounds shown in Table 6 and the processing speed was decreased by 0.05 round every day. The evaluation results are shown in Table 6.

**Table 6**

| Compound | Minimum Reflection Density Difference (ΔB) | Maximum Reflection Density Difference (ΔR) | Amount of Residual Silver (g/m²) |
|---|---|---|---|
| - | 0.04 | -0.04 | 0.03 |
| Methylsulfonic acid | 0.04 | -0.03 | 0.03 |
| II-1 | 0.02 | -0.01 | 0.01 |
| II-2 | 0.02 | -0.01 | 0.01 |
| II-14 | 0.02 | -0.01 | 0.01 |
| III-6 | 0.02 | -0.01 | 0.01 |
| III-8 | 0.02 | -0.01 | 0.01 |
| III-14 | 0.02 | -0.01 | 0.01 |

It can be understood from Table 6 that the effect of the invention can be demonstrated much better by adding aromatic compounds having a sulfonic acid group or aromatic compounds having a sulfate group to the color developer used in the processing according to the invention.

### Example 8

The procedure of Example 1 was repeated, except that the replenishing rate of the bleach-fixer was changed to the following processing conditions, and that the processing speed was changed to 0.03 round per day.

| Processing Condition No. | Replenishing Rate (ml/m²) |
|---|---|
| 1 | 200 |
| 2 | 120 |
| 3 | 100 |
| 4 | 50 |

The evaluation results are set forth in Table 7.

As is apparent from Table 7, the effect of the invention becomes more conspicuous as the replenishing rate of the bleach-fixer decreases, and the effect can be dramatically demonstrated when the replenishing rate is less than 120 ml/m².

### Example 9

The procedure of Example 2 was repeated, except that the bleach-fixing time was changed to the following processing conditions, and that the processing speed was changed to 0.03 round per day.

The evaluation results are shown in Table 8.

| Processing Condition No. | Processing Time (sec) |
|---|---|
| 1 | 45 |
| 2 | 35 |
| 3 | 30 |
| 4 | 25 |

As is apparent from Table 8, the effect of the invention becomes more conspicuous as the bleach-fixing time becomes shorter, and the effect can be best brought out when the bleach-fixing time is less than 30 seconds.

## Claims

1. A method for processing a silver halide color photographic light-sensitive material comprising the steps of developing a silver halide color photographic light-sensitive material comprising silver halide grains having a silver chloride content of not less than 80 mole % with a color developer containing a compound represented by the following Formula I wherein L is a substituted or unsubstituted alkylene group; A is a carboxyl group, a sulfo group, a phosphono group, a phosphinic acid group, hydroxyl group, an amino group, an ammonio group, a carbamoyl or a sulfamoyl group, in which said amino group, ammonio group, carbamoyl group and sulfamoyl group each may have an alkyl group as a substituent; R is a hydrogen atom or a substituted or unsubstituted alkyl group; or a monosaccharide
and bleach-fixing said light-sensitive material with a bleach-fixer,
containing a ferric complex salt of aminopolycarboxylic acid selected from the following Group 1 and an aliphatic dibasic acid selected from the following Group 2;
Group 1
Ferric ethylenediaminetetraacetate,
Ferric ethylenetriaminepentaacetate,
Ferric trans-1,2-cyclohexanediaminetetraacetate,
Ferric β-alaninediacetate,
Ferric ethylenediaminedisuccinate,
Ferric nitrylotriacetate,
Ferric N-hydroxyethylethylenediaminetriacetate and
Ferric glycoletherdiaminetetraacetate;
Group 2
Oxalic acid,
Succinic acid,
Maleic acid,
Fumaric acid, and
Adipic acid.

2. The method of claim 1, wherein said compound represented by Formula I is contained in said color developer in an amount of from 1.5 x 10⁻³ mol to 1.5 x 10⁻¹ mol per liter.

3. The method of claim 2, wherein said compound represented by Formula I is contained in said color developer in an amount of from 3.0 x 10⁻³ mol to 9.0 x 10⁻² mol per liter.

4. The method of claim 1, 2 or 3, wherein said monosaccharide is glyceraldehyde, dihydroxyacetone, dimer of dihydroxyacetone, D-erythrose, L-erythrose, D-threose, L-threose, D-ribose, L-ribose, D-arabinose, L-arabinose, D-xylose, L-xylose, D-lyxose, L-lyxrose, D-xylilose, L-xylulose, D-ribulose, L-ribulose, 2-dioxy-D-ribose, D-allose, L-allose, D-altrose, L-altrose, D-glucose, L-glucose, D-mannose, L-mannose, D-gulose, L-gulose, D-idose, L-idose, D-galactose, L-galactose, D-talose, L-talose, D-quinovose, digitalose, digitoxose, cymarose, D-sorbose, L-sorbose, D-tagatose, D-fucose, L-fucose, 2-dioxy-D-glucose, D-psicose, D-fructose, L-fructose, L-rhamnose, D-glucosamine, D-galactosamine, D-mannosamine, D-glycero-D-galactoheptose, D-glycero-D-mannoheptose, D-glycero-L-mannoheptose, D-glycero-guloheptose, D-glycero-D-idoheptose, D-glycero-L-glucoheptose, D-glycero-L-taloheptose, D-altroheptulose, D-mannoheptulose, D-altro-3-heptulose, D-glucronic acid, L-glucronic acid or N-acetyl-D-glucosamine.

5. The method of claim 4, wherein said monosaccharide is glyceraldehyde, D-ribose, L-ribose, D-arabinose, L-arabinose, D-xylose, L-xylose, D-ribulpse, 2-deoxy-D-ribose, D-allose, D-glucose, L-glucose, D-mannose, L-mannose, D-galactose, L-galactose, D-sorbose, L-sorbose, D-fructose, L-fructose, D-glucosamine, D-glucronic acid or N-acetyl-D-glucosamine.

6. The method of claim 5, wherein said monosaccharide is glyceraldehyde, D-ribose, L-ribose, D-sorbose, L-sorbose, D-fructose, L-fructose or D-glucosamine.

7. The method of claims 1 or 2 to 6, wherein said monosaccharide is contained in said color developer in an amount of from 1.5 x 10⁻³ mol to 1.5 x 10⁻¹ mol per liter.

8. The method of claim 7, wherein said monosaccharide is contained in said color developer in an amount of from 3.0 x 10⁻³ mol to 9.0 x 10⁻² mol per liter.

9. The method of claim 8, wherein said monosaccharide is contained in said color developer in an amount of from 4.5 x 10⁻³ mol to 6.0 x 10⁻² mol per liter.

10. The method of claims 1 or 2 to 9, wherein said color developer further contains a compound represented by Formula II or III: wherein A, B, C, D, E and F are each independently a -SO₃M group, -OSO₃M group, a hydrogen atom, a halogen atom or a saturated or unsaturated monovalent hydrocarbon group provided that at least one of groups represented by A, B, C, D, E and F is a -SO₃M group or -OSO₃M group, in which M is a hydrogen atom, an alkali metal atom or an ammonium group, wherein G, H, I, J, K, L, M and N are each independently a -SO₃M group, -OSO₃M group, a hydrogen atom, a halogen atom or a saturated or unsaturated monovalent hydrocarbon group provided that at least one of groups represented by G, H, I, J, K, L, M and N is a -SO₃M group or -OSO₃M group, in which M is a hydrogen atom, an alkali metal atom or an ammonium group.

11. The method of claim 10, wherein said compound represented by Formula II or III is contained in said color developer in an amount of not less than 5 g per liter.

12. The method of claim 11, wherein said compound represented by Formula II or III is contained in said color developer in an amount of from 10 g to 200 g per liter.

13. The method of claims 1 or 2 to 12, wherein said aliphatic dibasic acid is contained in said bleach-fixer in an amount of from 1.5 x 10 ⁻² mol to 8.5 x 10 ⁻¹ mol per liter.

14. The method of claim 13, wherein said aliphatic dibasic acid is contained in said bleach-fixer in an amount of from 8.0 x 10 ⁻² mol to 4.3 x 10 ⁻¹ mol per liter.

15. The method of claims 1 or 2 to 14, wherein said ferric complex of aminopolycarboxylic acid is contained in said bleach-fixer in an amount of not less than 0.01 mol per liter.

16. The method of claim 15, wherein said ferric complex of aminopolycarboxylic acid is contained in said bleach-fixer in an amount of from 0.03 mol to 0.3 mol per liter.

17. The method of claim 16, wherein said ferric complex of aminopolycarboxylic acid is contained in said bleach-fixer in an amount of from 0.05 mol to 0.25 mol per liter.

18. The method of claims 1 or 2 to 17, wherein said silver halide grains have a silver chloride content of not less than 90 mol %.

19. The method of claim 18, wherein said silver halide grains have a silver chloride content of not less than 95 mol %.

20. The method of claim 19, wherein said silver halide grains have a silver chloride content of not less than 98 mol %.

21. The method of claims 1 or 2 to 20, wherein said bleach-fixing step by said bleach-fixer is carried out for a time of from 35 seconds to 55 seconds.

22. The method of claim 21, wherein said bleach fixer is replenished with a bleach-fixer replenisher in a rate of 30 ml to 120 ml per square meter of said light-sensitive material processed by said bleach-fixer.

23. The method of claims 1 to 20, wherein said bleach-fixing step by said bleach-fixer is carried out for a time of from 5 seconds to 30 seconds.

24. The method of claim 23, wherein said bleach fixer is replenished with a bleach-fixer replenisher in a rate of 50 ml to 250 ml per square meter of said light-sensitive material processed by said bleach-fixer.

## Patentansprüche

1. Verfahren zur Entwicklung eines farbphotographischen, lichtempfindlichen Silberhalogenid-Materials, umfassend die Stufen Entwicklung eines lichtempfindlichen, farbphotographischen Silberhalogenid-Materials, umfassend Silberhalogenid-Körner mit einem Silberchlorid-Gehalt von nicht weniger als 80 Mol-% mit einem Farbentwickler, der eine durch die folgende Formel (1) dargestellte Verbindung enthält wobei L eine substituierte oder unsubstituierte Alkylengruppe ist; A eine Carboxylgruppe, eine Sulfogruppe, eine Phosphonogruppe, eine Phosphinsäuregruppe, eine Hydroxylgruppe, eine Aminogruppe, eine Ammoniogruppe, eine Carbamoylgruppe oder eine Sulfamoylgruppe ist, wobei die Aminogruppe, Ammoniogruppe, Carbamoylgruppe oder Sulfamoylgruppe jeweils eine Alkylgruppe als Substituent aufweisen kann; R ein Wasserstoffatom oder eine substituierte oder unsubstituierte Alkylgruppe ist; oder ein Monosaccharid enthält, und
Bleich-Fixieren des lichtempfindlichen Materials mit einem Bleich-Fixierer,
der ein Eisen-(III)-Komplexsalz einer Aminopolycarbonsäure enthält, das ausgewählt wird aus der folgenden Gruppe 1, und eine aliphatische, dibasische Säure, die aus der folgenden Gruppe 2 ausgewählt wird;
Gruppe 1
Eisen(III)ethylendiamintetraacetat,
Eisen(III)ethylentriaminpentaacetat,
Eisen(III)-trans-1,2-cyclohexandiamintetraacetat,
Eisen(III)-β-alanindiacetat,
Eisen(III)ethylendiamindisuccinat,
Eisen(III)nitrilotriacetat,
Eisen(III)-N-hydroxyethylethylendiamintriacetat und
Eisen(III)glycoletherdiamintetraacetat;
Gruppe 2
Oxalsäure,
Bernsteinsäure,
Maleinsäure,
Fumarsäure und
Adipinsäure.

2. Verfahren nach Anspruch 1, wobei die durch Formel I dargestellte Verbindung im Farbentwickler in einer Menge von 1,5 x 10⁻³ Mol bis 1,5 x 10⁻¹ pro Liter enthalten ist.

3. Verfahren nach Anspruch 2, wobei die durch Formel I dargestellte Verbindung im Farbentwickler in einer Menge von 3,0 x 10⁻³ Mol bis 9,0 x 10⁻² Mol pro Liter enthalten ist.

4. Verfahren nach Anspruch 1, 2 oder 3, wobei das Monosaccharid Glycerinaldehyd, Dihydroxyaceton, Dimer von Dihydroxyaceton, D-Erythrose, L-Erythrose, D-Threose, L-Threose, D-Ribose, L-Ribose, D-Arabinose, L-Arabinose, D-Xylose, L-Xylose, D-Lyxose, L-Lyxose, D-Xylulose, L-Xylulose, D-Ribulose, L-Ribulose, 2-Deoxy-D-ribose, D-Allose, L-Allose, D-Altrose, L-Altrose, D-Glucose, L-Glucose, D-Mannose, L-Mannose, D-Gulose, L-Gulose, D-Idose, L-Idose, D-Galactose, L-Galactose, D-Talose, L-Talose, D-Chinovose, Digitalose, Digitoxose, Cymarose, D-Sorbose, L-Sorbose, D-Tagatose, D-Fucose, L-Fucose, 2-Deoxy-D-glucose, D-Psicose, D-Fructose, L-Fructose, L-Rhamnose, D-Glucosamin, D-Galactosamin, D-Mannosamin, D-Glycero-D-galactoheptose, D-Glycero-D-mannoheptose, D-Glycero-L-mannoheptose, D-Glycero-D-guloheptose, D-Glycero-D-idoheptose, D-Glycero-L-glucoheptose, D-Glycero-L-taloheptose, D-Altroheptulose, D-Mannoheptulose, D-Altro-3-heptulose, D-Glucuronsäure, L-Glucuronsäure oder N-Acetyl-D-glucosamin ist.

5. Verfahren nach Anspruch 4, wobei das Monosaccharid Glycerinaldehyd, D-Ribose, L-Ribose, D-Arabinose, L-Arabinose, D-Xylose, L-Xylose, D-Ribulose, 2-Deoxy-D-ribose, D-Allose, D-Glucose, L-Glucose, D-Mannose, L-Mannose, D-Galactose, L-Galactose, D-Sorbose, L-Sorbose, D-Fructose, L-Fructose, D-Glucosamin, D-Glucuronsäure oder N-Acetyl-D-glucosamin ist.

6. Verfahren nach Anspruch 5, wobei das Monosaccharid Glycerinaldehyd, D-Ribose, L-Ribose, D-Sorbose, L-Sorbose, D-Fructose, L-Fructose oder D-Glucosamin ist.

7. Verfahren nach Ansprüchen 1 oder 2 bis 6, wobei das Monosaccharid im Farbentwickler in einer Menge von 1,5 x 10⁻³ Mol bis 1,5 10⁻¹ Mol pro Liter enthalten ist.

8. Verfahren nach Anspruch 7, wobei das Monosaccharid im Farbentwickler in einer Menge von 3,0 x 10⁻³ Mol bis 9,0 x 10⁻² pro Liter enthalten ist.

9. Verfahren nach Anspruch 8, wobei das Monosaccharid im Farbentwickler in einer Menge von 4,5 x 10⁻³ Mol bis 6,0 x 10⁻² Mol pro Liter enthalten ist.

10. Verfahren nach Ansprüchen 1 oder 2 bis 9, wobei der Farbentwickler darüber hinaus eine durch Formel II oder III dargestellte Verbindung enthält: wobei A, B, C, D, E und F jeweils unabhängig eine -SO₃M-Gruppe, - OSO₃M-Gruppe, ein Wasserstoffatom, ein Halogenatom oder eine gesättigte oder ungesättigte monovalente Kohlenwasserstoffgruppe darstellen, vorausgesetzt, daß mindestens eine der durch A, B, C, D, E und F dargestellten Gruppen eine -SO₃M-Gruppe oder -OSO₃M-Gruppe ist, wobei M ein Wasserstoffatom, ein Alkalimetallatom oder eine Ammoniumgruppe ist wobei G, H, I, J, K, L, M und N jeweils unabhängig eine -SO₃M-Gruppe, -OSO₃M-Gruppe, ein Wasserstoffatom, ein Halogenatom oder eine gesättigte oder ungesättigte monovalente Kohlenwasserstoffgruppe darstellen, vorausgesetzt, daß mindestens eine der durch G, H, I, J, K, L, M und N dargestellten Gruppen eine -SO₃M-Gruppe oder -OSO₃M-Gruppe ist, wobei M ein Wasserstoffatom, ein Alkalimetallatom oder eine Ammoniumgruppe ist.

11. Verfahren nach Anspruch 10, wobei die durch Formel II oder III dargestellte Verbindung im Farbentwickler in einer Menge von nicht weniger als 5 g/Liter enthalten ist.

12. Verfahren nach Anspruch 11, wobei die durch Formel II oder III dargestellte Verbindung im Farbentwickler in einer Menge von 10 g bis 200 g pro Liter enthalten ist.

13. Verfahren nach Ansprüchen 1 oder 2 bis 12, wobei die aliphatische, dibasische Säure im Bleich-Fixierer in einer Menge von 1,5 x 10⁻² Mol bis 8,5 x 10⁻¹ Mol pro Liter enthalten ist.

14. Verfahren nach Anspruch 13, wobei die aliphatische, dibasische Säure im Bleich-Fixierer in einer Menge von 8,0 x 10⁻² Mol bis 4,3 x 10⁻¹ Mol pro Liter enthalten ist.

15. Verfahren nach Ansprüchen 1 oder 2 bis 14, wobei der Eisen-(III)-Komplex der Aminopolycarbonsäure im Bleich-Fixierer in einer Menge von nicht weniger als 0,01 Mol pro Liter enthalten ist.

16. Verfahren nach Anspruch 15, wobei der Eisen-(III)-Komplex der Aminopolycarbonsäure im Bleich-Fixierer in einer Menge von 0,03 Mol bis 0,3 Mol pro Liter enthalten ist.

17. Verfahren nach Anspruch 16, wobei der Eisen-(III)-Komplex der Aminopolycarbonsäure im Bleich-Fixierer in einer Menge von 0,05 Mol bis 0,25 Mol pro Liter enthalten ist.

18. Verfahren nach Ansprüchen 1 oder 2 bis 17, wobei die Silberhalogenid-Körner einen Silberchlorid-Gehalt von nicht weniger als 90 Mol-% aufweisen.

19. Verfahren nach Anspruch 18, wobei die Silberhalogenid-Körner einen Silberchlorid-Gehalt von nicht weniger als 95 Mol-% aufweisen.

20. Verfahren nach Anspruch 19, wobei die Silberhalogenid-Körner einen Silberchlorid-Gehalt von nicht weniger als 98 Mol-% aufweisen.

21. Verfahren nach Ansprüchen 1 oder 2 bis 20, wobei der Bleich-Fixierungs-Schritt mit dem Bleich-Fixierer in einer Zeit von 35 Sekunden bis 55 Sekunden durchgeführt wird.

22. Verfahren nach Anspruch 21, wobei der Bleich-Fixierer mit einem Bleich-Fixierungs-Wiederauffüller in einer Geschwindigkeit von 30 ml bis 120 ml pro m² des mit dem Bleich-Fixierer entwickelten lichtempfindlichen Materials wiederaufgefüllt wird.

23. Verfahren nach Ansprüchen 1 bis 20, wobei der Bleich-Fixierungs-Schritt mit dem Bleich-Fixierer in einer Zeit von 5 Sekunden bis 30 Sekunden durchgeführt wird.

24. Verfahren nach Anspruch 23, wobei der Bleich-Fixierer mit einem Bleich-Fixierungs-Wiederauffüller in einer Geschwindigkeit von 50 ml bis 250 ml pro m² des mit dem Bleich-Fixierer entwickelten lichtempfindlichen Materials wiederaufgefüllt wird.

## Revendications

1. Procédé de traitement d'un matériau photographique couleur sensible à la lumière à base d'halogénure d'argent, comprenant les étapes consistant à développer un matériau photographique couleur sensible à la lumière à base d'halogénure d'argent comprenant des grains d'halogénure d'argent ayant une teneur en chlorure d'argent de pas moins de 80% en moles avec un développateur couleur contenant un composé représenté par la formule I suivante dans laquelle L est un groupe alkylène substitué ou non substitué; A est un groupe carboxyle, un groupe sulfo, un groupe phosphono, un groupe acide phosphinique, un groupe hydroxyle, un groupe amino, un groupe ammonio, un groupe carbamoyle ou sulfamoyle, dans lequel lesdits groupe amino, groupe ammonio, groupe carbamoyle et groupe sulfamoyle peuvent porter chacun un groupe alkyle comme substituant; R est un atome d'hydrogène ou un groupe alkyle substitué ou non substitué; ou un monosaccharide;
et blanchiment-fixage dudit matériau sensible à la lumière avec un blanchisseur-fixateur, contenant un sel complexe ferrique d'acide aminopolycarboxylique choisi dans le groupe 1 suivant et un diacide aliphatique choisi dans le groupe 2 suivant;
Groupe 1
éthylènediaminetétraacétate ferrique,
éthylènetriaminepentaacétate ferrique,
trans-1,2-cyclohexanediaminetétraacétate ferrique,
β-alaninediacétate ferrique,
éthylènediaminedisuccinate ferrique,
nitrilotriacétate ferrique,
N-hydroxyéthyléthylènediaminetriacétate ferrique, et glycolétherdiaminetétraacétate ferrique;
Groupe 2
acide oxalique,
acide succinique,
acide maléique,
acide fumarique, et
acide adipique.

2. Procédé selon la revendication 1, dans lequel ledit composé représenté par la formule I est contenu dans ledit développateur couleur en une quantité de 1,5 x 10⁻³ mole à 1,5 x 10⁻¹ mole par litre.

3. Procédé selon la revendication 2, dans lequel ledit composé représenté par la formule I est contenu dans ledit développateur couleur en une quantité de 3,0 x 10⁻³ mole à 9,0 x 10⁻² mole par litre.

4. Procédé selon la revendication 1, 2 ou 3, dans lequel ledit monosaccharide est le glycéraldéhyde, la dihydroxyacétone, un dimère de dihydroxyacétone, le 3-érythrose, le L-érythrose, le D-thréose, le L-thérose, le D-ribose, le L-ribose, le D-arabinose, le L-arabinose, le D-xylose, le L-xylose, le D-lyxose, le L-lyxose, le D-xylilose, le L-xylilose, le D-ribulose, le L-ribulose, le 2-dioxy-D-ribose, le D-allose, le L-allose, le D-altrose, le L-altrose, le D-glucose, le L-glucose, le D-mannose, le L-mannose, le D-gulose, le L-gulose, le D-idose, le L-idose, le D-galactose, le L-galactose, le D-talose, le L-talose, le D-quinovose, le digitalose, le digitoxose, le cymarose, le D-sorbose, le L-sorbose, le D-tagatose, le D-fucose, le L-fucose, le 2-dioxy-D-glucose, le D-psicose, le D-fructose, le L-fructose, le L-rhamnose, la D-glucosamine, la D-galactosamine, la D-mannosamine, le D-glycéro-D-galactoheptose, le D-glycéro-D-mannoheptose, le D-glycéro-L-mannoheptosé, le D-glycéro-guloheptose, le D-glycéro-D-idoheptose, le D-glycéro-L-glucoheptose, le D-glycéro-L-taloheptose, le D-altroheptulose, le D-mannoheptulose, le D-altro-3-heptulose, l'acide D-glucuronique, l'acide L-glucuronique ou la N-acétyl-D-glucosamine.

5. Procédé selon la revendication 4, dans lequel ledit monosaccharide est le glycéraldéhyde, le D-ribose, le L-ribose, le D-arabinose, le L-arabinose, le D-xylose, le L-xylose, le D-ribulose, le 2-désoxy-D-ribose, le D-allose, le D-glucose, le L-glucose, le D-mannose, le L-mannose, le D-galactose, le L-galactose, le D-sorbose, le L-sorbose, le D-fructose, le L-fructose, la D-glucosamine, l'acide D-glucuronique ou la N-acétyl-D-glucosamine.

6. Procédé selon la revendication 5, dans lequel ledit monosaccharide est le glycéraldéhyde, le D-ribose, le L-ribose, le D-sorbose, le L-sorbose, le D-fructose, le L-fructose ou la D-glucosamine.

7. Procédé selon les revendications 1 ou 2 à 6, dans lequel ledit monosaccharide est contenu dans ledit développateur couleur en une quantité de 1,5 x 10⁻³ mole à 1,5 x 10⁻¹ mole par litre.

8. Procédé selon la revendication 7, dans lequel ledit monosaccharide est contenu dans ledit développateur couleur en une quantité de 3,0 x 10⁻³ mole à 9,0 x 10⁻² mole par litre.

9. Procédé selon la revendication 8, dans lequel ledit monosaccharide est contenu dans ledit développateur couleur en une quantité de 4,5 x 10⁻³ mole à 6,0 x 10⁻² mole par litre.

10. Procédé selon les revendications 1 ou 2 à 9, dans lequel ledit développateur couleur contient, en outre, un composé représenté par la formule II ou III: dans laquelle A, B, C, D, E et F sont chacun, indépendamment, un groupe -SO₃M, un groupe -OSO₃M, un atome d'hydrogène, un atome d'halogène ou un groupe hydrocarboné monovalent, saturé ou insaturé, pourvu qu'au moins un des groupes représentés par A, B, C, D, E et F soit un groupe -SO₃M ou un groupe -OSO₃M, où M est un atome d'hydrogène, un atome de métal alcalin ou un groupe ammonium; dans laquelle G, H, I, J, K, L, M et N sont chacun, indépendamment, un groupe -SO₃M, un groupe -OSO₃M, un atome d'hydrogène, un atome d'halogène ou un groupe hydrocarboné monovalent, saturé ou insaturé, pourvu qu'au moins un des groupes représentés par G, H, I, J, K, L, M et N soit un groupe -SO₃M ou un groupe -OSO₃M, où M est un atome d'hydrogène, un atome de métal alcalin ou un groupe ammonium.

11. Procédé selon la revendication 10, dans lequel ledit composé représenté par la formule II ou III est contenu dans ledit développateur couleur en une quantité de pas moins de 5 g par litre.

12. Procédé selon la revendication 11, dans lequel ledit composé représenté par la formule II ou III est contenu dans ledit développateur couleur en une quantité de 10 g à 200 g par litre.

13. Procédé selon les revendications 1 ou 2 à 12, dans lequel ledit diacide aliphatique est contenu dans ledit blanchisseur-fixateur en une quantité de 1,5 x 10⁻² mole à 8,5 x 10⁻¹ mole par litre.

14. Procédé selon la revendication 13, dans lequel ledit diacide aliphatique est contenu dans ledit blanchisseur-fixateur en une quantité de 8,0 x 10⁻² mole à 4,3 x 10⁻¹ mole par litre.

15. Procédé selon les revendications 1 ou 2 à 14, dans lequel ledit complexe ferrique d'acide aminopolycarboxylique est contenu dans ledit blanchisseur-fixateur en une quantité de pas moins de 0,01 mole par litre.

16. Procédé selon la revendication 15, dans lequel ledit complexe ferrique d'acide aminopolycarboxylique est contenu dans lequel blanchisseur-fixateur en une quantité de 0,03 mole à 0,3 mole par litre.

17. Procédé selon la revendication 16, dans lequel ledit complexe ferrique d'acide aminopolycarboxylique est contenu dans ledit blanchisseur-fixateur en une quantité de 0,05 mole à 0,25 mole par litre.

18. Procédé selon les revendications 1 ou 2 à 17, dans lequel lesdits grains d'halogénure d'argent ont une teneur en chlorure d'argent de pas moins de 90% en moles.

19. Procédé selon la revendication 18, dans lequel lesdits grains d'halogénure d'argent ont une teneur en chlorure d'argent de pas moins de 95% en moles.

20. Procédé selon la revendication 19, dans lequel lesdits grains d'halogénure d'argent ont une teneur en chlorure d'argent de pas moins de 98% en moles.

21. Procédé selon les revendications 1 ou 2 à 20, dans lequel ladite étape de blanchiment-fixage par ledit blanchisseur-fixateur est réalisée pendant une durée de 35 secondes à 55 secondes.

22. Procédé selon la revendication 21, dans lequel ledit blanchisseur-fixateur est régénéré avec un apport de blanchisseur-fixateur à une vitesse de 30 mL à 120 mL par mètre carré dudit matériau sensible à la lumière traité par ledit blanchisseur-fixateur.

23. Procédé selon les revendications 1 à 20, dans lequel ladite étape de blanchiment-fixage par ledit blanchisseur-fixateur est réalisée pendant une durée de 5 secondes à 30 secondes.

24. Procédé selon la revendication 23, dans lequel ledit blanchisseur-fixateur est régénéré avec un apport de blanchisseur-fixateur à une vitesse de 50 mL à 250 mL par mètre carré dudit matériau sensible à la lumière traité par ledit blanchisseur-fixateur.
